# EUROPEAN PATENT SPECIFICATION

(11) **EP 0 228 756 B1**
(45) Date of publication and mention of the grant of the patent: **16.05.1990**
(21) Application number: 86300108.7
(22) Date of filing: 08.01.1986
(51) Int. Cl.: C22C 38/14, C22C 38/12

(54) **Extra low carbon steel sheets**
Stahlbleche mit sehr niedrigem Kohlenstoffgehalt
Tôles en acier à très basse teneur en carbone

(43) Date of publication of application: 15.07.1987
(73) Proprietor: KAWASAKI STEEL CORPORATION, Chuo-Ku, Kobe-City Hyogo 651 (JP)
(72) Inventor: Hashimoto, Osamu, 1, Kawasaki-Cho Chiba City Chiba Pref. (JP); Sakata, Kei, 1, Kawasaki-Cho Chiba City Chiba Pref. (JP); Ishii, Chikako, 1, Kawasaki-Cho Chiba City Chiba Pref. (JP); Gotoh, Minari, 1, Kawasaki-Cho Chiba City Chiba Pref. (JP)
(74) Representative: Overbury, Richard Douglas

(56) References cited:
- EP-A- 0 171 208
- DE-A- 2 362 658
- US-A- 3 765 874
- JAPANESE PATENT ABSTRACTS, vol. J6-M, Week 8612, page 17, no. JP 86 078 320 (KAWASAKI STEEL K.K.) 06-02-1986

## Description

This invention relates to extra low carbon steel sheets having good chemical conversion characteristics, and more particularly to providing an improvement in the phosphatability of carbonitride- containing extra low carbon steel sheets.

Extra low carbon steel sheets containing Ti have excellent properties such as low yield point, high ductility and the like in view of their mechanical properties (as described in Japanese Patent Application Publication No. 44-18,066). However, if it is intended to use the above steel sheet as, for example, an outer panel for an automotive vehicle, there is the problem that the phosphatability is poor and hence its use is considerably restricted.

This results mainly from the fact that the surface of the steel sheet is covered with an oxide film of Ti. The Ti, which is abundantly existent in the steel sheet, concentrates in the surface of the steel sheet during the long time for which it is maintained at high temperature after the coiling following the hot rolling or during the recrystallization annealing after the cold rolling. This titanium reacts with oxygen in the atmosphere to form an oxide film which has a bad influence.

With a view to preventing the above drawback, there is known a method wherein Mn, S, P and the like are concentrated on the surface of the steel sheet (as described, for example, in Japanese Patent laid open No. 59-74,259) and so on. However, as the amounts of the above three elements increase, the physical properties of the steel are degraded, so that it is useless to attempt to provide good mechanical properties by decreasing the carbon content to an extremely low amount and adding Ti.

It is, therefore, an object of the invention to provide steel sheets having good phosphatability without causing the material degradation as mentioned above.

US-A-3 765 874 discloses a low carbon vacuum degassed steel having good formability and good non-aging properties. The steel contains from 0.002 to 0.020% carbon, up to 0.60% manganese, from greater than 0.025 to 0.12% columbium (niobium), optionally titanium in an amount of from 0.015 to 0.12%, optionally zirconium in an amount of from 0.028 to 0.18%, up to 0.008% nitrogen, up to 0.010% total oxygen, up to 0.035% sulphur, and up to 0.045% total aluminium. The carbon and nitrogen are fixed by the Nb, Ti and Zr at the hot rolling stage so as to obtain cold rolled sheets having good formability and non-aging properties. There is no suggestion that the steel has improved phosphatability.

EP-A-0 171 208 (designating DE, FR, GB, IT and SE) is concerned with steel sheets suitable for the outer panels of automobiles having good formability. The steel contains from 0.0005 to 0.015% carbon, not more than 1.0% silicon, not more than 1.0% Mn, not more than 0.15% P, 0.005 to 0.100% Al, not more than 0.003% S, not more than 0.004% N provided that S + N is not more than 0.005%, Ti in specified amounts depending on the C, N and S contents, and optionally not more than 0.05% Nb and not more than 0.0050% B. Both the N and S contents are severely restricted in order to leave solute C for strain aging. There is no suggestion that the addition of Ti and Nb is useful for improving phosphatability.

DE-A-2 362 658 discloses a method of manufacturing a steel sheet having good press formability by subjecting a killed steel to warm rolling such that the finishing temperature is 750°C or less and thereafter carrying out a recrystallisation treatment. The killed steel is composed of not more than 0.10% C, 0.05% to 1.0% Mn, 0.05% to 0.15% Al, at least one of Ti, Nb and Zr with the remainder being Fe and impurities. The value of is more than the percentage of carbon present in the steel. There is no suggestion that the steel has improved phosphatability.

According to the present invention, there is provided an extra low carbon steel sheet formed from a composition consisting of carbon, nitrogen, silicon, manganese, aluminium, titanium and niobium with the balance being iron and incidental impurities including sulphur characterised in that the sheet is a phosphated sheet and in that the carbon is present in an amount of not more than 0.01 wt%, the nitrogen is present in an amount of not more than 0.01 wt%, the silicon is present in an amount of not more than 0.15 wt%, the manganese is present in an amount of not more than 0.6 wt%, the aluminium is present in an amount of not more than 0.10 wt%, the titanium is present in an amount not less than 4.0x([C]+[N]), and the niobium is present within a range of 1/6x[Ti] to 31/4x[C].

For a better understanding of the invention and to show how the same may be carried out, reference will now be made, by way of example, to the accompanying drawing which shows a graph illustrating the relationship between the amounts of Ti and Nb and the pin hole area ratio (PHE).

The invention is based on the phenomenon found during an investigation of the mechanical properties and phosphatability of Nb and/or Ti-containing steel.

Namely, each of the steels having the chemical composition shown in the following Table 1, wherein variable amounts of Nb were added to a steel containing an amount of Ti larger than a specified total amount of C and N, was melted in a laboratory and shaped into a slab, which was then hot rolled, cold rolled, electrolytically degreased and continuously annealed at 830°C for 20 seconds. Next, the mechanical properties and phosphatability of the resulting steel sheet were examined.

The phosphatability was estimated by the pin hole area ratio (hereinafter abbreviated as PHE) when the steel sheet was degreased, rinsed with water, phosphated and subjected to a pin hole test as mentioned IMM.

In the pin hole test, the portion of the surface of the steel sheet which was not covered by phosphate crystal coating was detected by sticking to the surface a filter paper impregnated with a reagent which develops a color by reaction with iron ion. The PHE was determined by image analysis.

Separately, it was confirmed that a PHE ≤ 3.0 corresponded to a good phosphatability.

In the single figure there is shown the relationship between the Ti and Nb amounts and the PHE, from which there was found the following. As the Ti amount increases, the PHE becomes higher whereas the PHE lowers as the Nb amount increases. In a steel containing a given amount of Ti, when the Nb amount is not less than 1/6 of the amount of Ti, the PHE becomes not more than 3, which corresponds to a good phosphatability.

Ti preferentially bonds to S, N and C in the steel to form precipitates, and at the same time concentrates in the surface of the steel to form an oxide film which degrades the phosphatability as previously mentioned. Therefore, when the amount of Ti added is sufficiently small, there is no problem with the phosphatability but the mechanical properties are unsatisfactory. However the phosphatability is degraded as the Ti amount is increased. According to the invention, it is necessary that the amount of Ti added is not less than 4 times the total amount of C and N in order to provide non-aging steel sheets.

On the other hand, the phosphatability is largely improved as the amount of Nb added increases. This is believed to be because the surface concentration of Ti is first suppressed with the increase of the Nb amount, so that Ti can not completely fix carbon unless a sufficiently excessive amount of Ti is added compared to the amounts of C, N and S in the steel. Thus Nb reacts with C to form NbC series precipitates on the surface of the steel sheet, which provide nuclei for the phosphate crystals.

Moreover, it is known that when the amount of solute carbon is not more than 0.005%, such solute carbon is included in the crystal grain boundary to provide a completely non-aging steel sheet.

However, when the Nb amount is excessive compared to the C amount, the phosphatability is degraded. Therefore, the Nb amount must be limited to not more than 31/4 times the C amount.

The reason why the amounts of C and N are limited to not more than 0.01 %, respectively, is to ensure the press formability and the mechanical properties. For the same reason as described above, the amounts of Mn and Si are limited to not more than 0.6% and not more than 0.15%, respectively. AI is accepted to be not more than 0.1 % when used as the deoxidizer in steel making. Moreover, the inevitable impurities are P and S, which are accepted to be not more than 0.15% and 0.02%, respectively, according to the invention.

The steel sheet according to the invention is manufactured by subjecting a steel of a particular chemical composition to continuous casting, hot rolling, cold rolling and annealing in the usual manner.

The following examples are given in order to illustrate the invention and are not intended as limitations thereof.

Each of the cold rolled steel sheets having the chemical compositions shown in the following Table 2 was manufactured by box annealing or continuous annealing.

The phosphatibility (PHE) and mechanical properties (Al, aging index, kg/mm²) were measured with respect to the resulting steel sheets and the results shown in the following Table 3 were obtained. Moreover, the phosphatic treatment was carried out with BT 3112 made by Japan Perkerizing K.K., adjusting to total acidity of 14.3 and free acidity of 0.5 at 55°C, and then spraying on the surface of the steel sheet for 120 seconds. The phosphatability was evaluated by the PHE as previously mentioned.

As can be seen from Table 3, when the Ti amount is less than 4 times the total amount of C and N (Steel sheet No. 5), Al is not zero, so that a so-called non-aging steel sheet cannot be obtained. Even when using a high grade, extra low carbon steel containing not more than 0.01% of each of carbon and nitrogen amounts, if the non-aging property can not be ensured, the application of the steel is restricted considerably. Therefore, the Ti amount must be not less than 4 times the total amount of C and N.

On the other hand, the phosphatability is degraded with an increase in the Ti amount but it is improved by adding Nb in an amount of not less than 1/6 of the Ti amount. When the Nb amount is less than 1/6 of the Ti amount (Steel sheet No. 6) or more than 31/4 of the C amount (Steel sheet No. 7), the PHE exceeds 3, and the phosphatability is degraded.

Even in the case of steels containing more than 0.01 % of C or N amount, the non-aging property can be obtained by the sufficient addition of Ti. In this case however, the yield strength becomes high and the elongation or ductility becomes poor. Thus there is no point in the addition of large amounts ofTi. For this reason, a large amount of Nb is also required to be added to improve the phosphatability. As a result, the mechanical properties of the steel are largely deteriorated (rise of yield point, reduction of elongation and the like). Therefore, the Nb amount is limited to 31/4 of C amount.

According to the invention, the remarkable improvement of phosphatability can be realized without causing a deterioration in the excellent properties of Ti-containing extra low carbon steel sheets.

## Claims (Claims for the following Contracting State(s) : s: FR DE GB SE)

1. A phosphated extra low carbon steel sheet formed from a composition consisting of carbon, nitrogen, silicon, manganese, aluminium, titanium and niobium with the balance b]eing iron and incidental impurities including sulphur characterised in that the carbon is present in an amount of not more than 0.01 wt%, the nitrogen is present in an amount of not more than 0.01 wt%, the silicon is present in an amount of not more than 0.15 wt%, the manganese is present in an amount of not more than 0.6 wt%, the aluminium is present in an amount of not more than 0.10 wt%, the titanium is present in an amount not less than 4.Ox([C]+[N]), the niobium is present within a range of 1/6x[Ti] to 31/4x[C], and the sulphur is present in an amount of more than 0.003 wt%.

2. A phosphated sheet as claimed in claim 1, wherein said incidental impurities include not more than 0.15 wt% of phosphorus.

3. A phosphated sheet as claimed in claim 1 or 2 wherein the sulphur content is not more than 0.02 wt%.

## Claims (Claims for the following Contracting State(s) : s: BE NL)

1. An extra low carbon steel sheet from a composition consisting of carbon, nitrogen, silicon, manganese, aluminium, titanium and niobium with the balance being iron and incidental impurities including sulphur characterised in that the sheet is a phosphated sheet and in that the carbon is present in an amount of not more than 0.01 wt%, the nitrogen is present in an amount of not more than 0.01 wt%, the silicon is present in an amount of not more than 0.15%, the manganese is present in an amount of not more than 0.6 wt%, the aluminium is present in an amount of not more than 0.10%, the titanium is present in an amount not less than 4.0x([C]+[N]), and the niobium is present within a range of 1/6x[Ti] to 31/4x[C].

2. An extra low carbon steel sheet as claimed in claim 1, wherein said incidental impurities include not more than 0.15 wt% of phosphorus and not more than 0.02 wt% of sulphur.

3. An extra low carbon steel sheet as claimed in claim 2 wherein the sulphur content is more than 0.003 wt%.

## Patentansprüche (Patentansprüche für folgende(n) Vertragsstaat(en) : DE FR GB SE)

1. Phosphatiertes Blech aus extra kohlenstoffarmem Stahl, gebildet aus einer Zusammensetzung, bestehend aus Kohlenstoff, Stickstoff, Silicium, Mangan, Aluminium, Titan und Niob, wobei der Rest Eisen und zufällige Verunreinigungen, einschließlich Schwefel sind, dadurch gekennzeichnet, daß der Kohlenstoff in einer Menge von nicht mehr als 0,01 Gew.-% anwesend ist, der Stickstoff in einer Menge von nicht mehr als 0,01 Gew.-% anwesend ist, das Silicium in einer Menge von nicht mehr 0,15 Gew.-% anwesend ist, das Mangan in einer Menge von nicht mehr als 0,6 Gew.-% anwesend ist, das Aluminium in einer Menge von nicht mehr als 0,10 Gew.-% anwesend ist, das Titan in einer Menge von nicht weniger als 4,0 x ([C] + [N]) anwesend ist, das Niob innerhalb eines Bereichs von 1/6 x [Ti] bis 31/4 x [C] vorliegt und der Schwefel in einer Menge von mehr als 0,003 Gew.-% vorliegt.

2. Phosphatiertes Blech nach Anspruch 1, worin die zufälligen Verunreinigungen nicht mehr als 0,15 Gew.-% Phosphor einschließen.

3. Phosphatiertes Blech nach Anspruch 1 oder 2, worin der Schwefel-Gehalt nicht größer als 0,02 Gew.- % ist.

## Patentansprüche (Patentansprüche für folgende(n) Vertragsstaat(en) : BE NL)

1. Blech aus extra kohlenstoffarmem Stahl, gebildet aus einer Zusammensetzung, bestehend aus Kohlenstoff, Stickstoff, Silicium, Mangan, Aluminium, Titan und Niob, wobei der Rest Eisen und zufällige Verunreinigungen, einschließlich Schwefel sind, dadurch gekennzeichnet, daß das Blech ein phosphatiertes Blech ist und daß der Kohlenstoff in einer Menge von nicht mehr als 0,01 Gew.-% anwesend ist, der Stickstoff in einer Menge von nicht mehr als 0,01 Gew.-% anwesend ist, das Silicium in einer Menge von nicht mehr 0,15 Gew.-% anwesend ist, das Mangan in einer Menge von nicht mehr als 0,6 Gew.-% anwesend ist, das Aluminium in einer Menge von nicht mehr als 0,10 Gew.-% anwesend ist, das Titan in einer Menge von nicht weniger als 4,0 x ([C] + [N]) anwesend ist und das Niob innerhalb eines Bereichs von 1/6 x [Ti] bis 31/4 x [C] vorliegt.

2. Blech aus extra kohlenstoffarmem Stahl nach Anspruch 1, worin die zufälligen Verunreinigungen nicht mehr als 0,15 Gew-% Phosphor und nicht mehr als 0,02 Gew.-% Schwefel einschließen.

3. Blech aus extra kohlenstoffarmem Stahl nach Anspruch 2, worin der Schwefel-Gehalt größer als 0,003 Gew.-% ist.

## Revendications (Revendications pour l'(les) Etat(s) contractant(s) suivant(s) : DE FR GB SE)

1. Tôle phosphatée à très basse teneur en carbone formée à partir d'une composition consistant en du carbone, de l'azote, du silicium, du manganèse, de l'aluminium, du titane et du niobium, le complément étant du fer et des impuretés accidentelles comprenant le soufre, caractérisée en ce que le carbone est présent en une quantité ne dépassant pas 0,01 % en poids, l'azote est présent en une quantité ne dépassant pas 0,01 % en poids, le silicium est présent en une quantité ne dépassant pas 0,15% en poids, le manganèse est présent en une quantité ne dépassant pas 0,6% en poids, l'aluminium est présent en une quantité ne dépassant ps 0.10% in poids le titane est présent en une quantité qui n'est pas inférieure à 40 x [C]t [N]), le niobium est présent en une quantité comprise entre 1/6 x [Ti] et 31/4 x [C], et le soufre est présent en une quantité ne dépassant pas 0,003% en poids.

2. Tôle phosphatée selon la revendication 1, dans laquelle les impuretés accidentelles ne comprennent pas plus de 0,15% en poids de phosphore.

3. Tôle phosphatée selon la revendication 1 ou 2, dans laquelle la teneur en soufre n'est pas supérieure à 0,02% en poids.

## Revendications (Revendications pour l'(les) Etat(s) contractant(s) suivant(s) : BE NL)

1. Tôle à très bass teneur en carbone formée d'une composition consistant en du carbone, de l'azote, du silicium, du manganèse, de l'aluminium, du titane et du niobium, le complément étant du fer et des impuretés accidentelles comprenant le soufre, caractérisée en ce que cette tôle est une tôle phosphatée et en ce que le carbone est présent en une quantité ne dépassant pas 0,01% en poids, l'azote est présent en une quantité ne dépassant pas 0,01 % en poids, le silicium est présent en une quantité ne dépassant pas 0,15% en poids, le manganèse est présent en une quantité ne dépassant pas 0,6% en poids, l'aluminium est présent en une quantité ne dépassant pas 0,10% en poids, le titane est présent en une quantité qui n'est pas inférieure à 4,0 x ([C] +t [N]) et le niobium est présent en une quantité comprise entre 1/6 x [Ti] a 31/4 x [C].

2. Tôle à très basse teneur en carbone selon la revendication 1, dans laquelle les impuretés accidentelles ne comprennent pas plus de 0,15% en poids de phosphore et pas plus de 0,02% en poids de soufre.

3. Tôle à très basse teneur en carbone selon la revendication 2, dans laquelle la teneur en soufre ne dépasse pas 0,003% en poids.
